# EUROPEAN PATENT APPLICATION

(11) **EP 0 646 673 A2**
(43) Date of publication of application: **05.04.1995**
(21) Application number: 94115399.1
(22) Date of filing: 29.09.1994
(51) Int. Cl.: D06P 1/00, D06P 1/52

(54) **Method of reversibly photochromic or thermochronic coloring by padding and colored product made thereby**

(30) Priority: 05.10.1993 JP 274884/93
(71) Applicant: MATSUI SHIKISO CHEMICAL CO., LTD, Yamashina-Ku, Kyoto-shi, Kyoto (JP)
(72) Inventor: Kitagawa, Yosuke, c/o Matsui Shikiso Chem. Co.,LTD, Kyoto-shi, Kyoto (JP); Hoshikawa, Ryuichi, c/o Matsui Shikiso Ch. Co.,LTD, Kyoto-shi, Kyoto (JP)
(74) Representative: Liedl, Christine, Dipl.-Chem.

(57) **Abstract**

A lengthy continuous textile product is serially treated with an aqueous liquid containing a thermoplastic resin and thermochromic and/or photochromic microcapsules having a volume-based median diameter of 0.5µ m to 15 µ m by padding. The textile product is colored with the reversibly color changing microcapsules without the tailing and reverse tailing phenomena.

## Description

The present invention relates to a method of coloring a lengthy continuous textile product with reversibly color changing microcapsules, and a colored product made thereby.

Previously, the present inventors proposed a method of efficiently coloring a lengthy continuous textile product with a reversibly color changing material wherein the reversibly color changing material is carried on the textile product by padding after the product is treated with a cationic nitrogenous compound (Japanese Patent Application No. 60959/1993).

Although the above-mentioned coloring method is very useful for industrial application in that reversibly color changing materials can be applied to textile products by padding, an approach that has been thought to be impossible for some reasons including longitudinally ununiform coloring, it involves multiple steps because of the necessity for a separate pretreatment with a nitrogenous cationic compound, a step not needed in ordinary practice of padding.

In addition, the nitrogenous cationic compound, originally used to prevent the reverse tailing phenomenon in padding operation, can result in the tailing phenomenon owing to excess acceleration of adhesion of non-vehicle components (i.e. components which are in the padding bath and are not vehicle or do not act as vehicle) such as reversibly color changing materials, depending on kind of textile product and kind of nitrogenous cationic compound.

The object of the present invention is to provide a method of uniformly and efficiently coloring a lengthy continuous textile product with reversibly color changing microcapsules by padding without the tailing and reverse tailing phenomena, and a colored product made thereby.

The present inventors found that the above-described tailing and reverse tailing phenomena occur with very strong dependency on the size of various particles which are non-vehicle components in the padding bath. Through further investigations, the inventors found it possible to use reversibly color changing microcapsules whose particle size fall within a particular range to obtain a reversibly color changing colored product uniformly colored with said microcapsules as a result of prevention of the reverse tailing phenomenon and also the tailing phenomenon even without pretreatment with a nitrogenous cationic compound, and developed the present invention. Accordingly, the coloring method of the present invention is characterized in that a lengthy continuous textile product is serially treated with an aqueous liquid containing a thermoplastic resin and thermochromic and/or photochromic microcapsules having a volume-based median diameter of 0.5µ m to 15 µ m by padding.

In case the volume-based median diameter of the thermochromic and/or photochromic microcapsules is under 0.5µ m, the color density of the colored product is too low to offer practical applicability because of the increased ratio of non-coloring components i.e. microcapsule-wall in the microcapsules, though the microcapsules are easily carried on the textile product so that at least the reverse tailing phenomenon is prevented.

If the volume-based median diameter of the thermochromic and/or photochromic microcapsules exceeds 15µ m, the reverse tailing phenomenon cannot be prevented, unless the textile product is pretreated with a nitrogenous cationic compound, not conforming to the object of the present invention. This is partially because the microcapsules tend to leave the textile product upon nipping. The above-mentioned volume-based median diameter can be determined easily using an instrument such as a laser diffraction/scattering particle size distribution analyzer.

According to the present invention, a lengthy continuous textile product can be colored very uniformly, both transversely and longitudinally, with reversibly color changing microcapsules by directly treating the textile product by padding without pretreatment with a nitrogenous cationic compound, provided that the volume-based median diameter of the reversibly color changing microcapsules falls within a particular range. In addition, the colored product thus obtained is as excellent as the original textile product in handling touch and appearance, and have excellent rubbing fastness and washing fastness. For this reason, the present invention significantly simplifies the previous process involving multiple stages due to the pretreatment with the nitrogenous cationic compound, to improve production efficiency; this effect, combined with avoidance of use of the nitrogenous cationic compound, offers significant reduction in the cost for producing reversibly color changing colored products.

The reversibly color changing microcapsules for the present invention include both thermochromic microcapsules, which show reversible color changes due to temperature changes, and photochromic microcapsules, which show reversible color changes according to the absence or presence of light irradiation, and also include microcapsules showing hysteresis in the color-changing cycle. It is of course possible to use one or more kinds of thermochromic microcapsules and photochromic microcapsules in combination, to obtain textile products with enriched color variation for additional commercial value.

Such microcapsules are exemplified as follows:
Examples of thermochromic microcapsules include fine particles prepared by encapsulating a conventional thermochromic material such as a two-component composition consisting of an acid developing substance such as the leuco dye for pressure/heat-sensitive copying paper, and an acidic substance capable of developing and eliminating the acid developing substance such as phenol; a three-component composition consisting of the above-described acid developing substance and acidic substance and an organic solvent such as an alcohol or an ester; or a mixed liquid crystal composition comprising a cholesteric liquid crystal, chiral nematic liquid crystal, etc., in a coat-forming polymer compound by a known method such as interfacial polymerization, in situ polymerization, in-liquid setting coating (orifice method), coacervation or spray drying, fine particles prepared by solid-dissolving the above-described thermochromic material in a polymer compound, and
fine particles of a material prepared by dispersing the above-described thermochromic material in a synthetic resin matrix.

Examples of photochromic microcapsules include fine particles of a material prepared by dispersing an organic photochromic compound such as the spiropyran, spiroxazine, naphthopyran or fulgide series in a synthetic resin matrix,
fine particles prepared by encapsulating such matrix particles in the above-described coat-forming polymer compound, and
fine particles prepared by encapsulating or solid-dissolving a solution or dispersion mixture of the above-described organic photochromic compound in a medium such as a hindered amine, hindered phenol, plasticizer, high boiling point solvent or synthetic resin, in the above-described coat-forming polymer compound.

The above-described microcapsules, singly or in combination of two or more kinds, are dispersed in water to form an aqueous liquid together with a thermoplastic resin.

Any thermoplastic resin can be used for the present invention, as long as it is known to serve as an adhesive component in padding bath, such as acrylic acid ester resin, methacrylic acid ester resin, vinyl acetate resin, polyurethane resin, polyester resin, styrene-butadiene latex, or polyolefin resin. Such thermoplastic resins, singly or in combination of two or more kinds, can be used in the form of an aqueous solution or emulsion.

The thermoplastic resin acts to adhere thermochromic and/or photochromic microcapsules on a textile product.

The thermoplastic resin used may be partially cross-linkable, or may be used in combination with another cross-linkable resin. In such cases, a cross-linking catalyst is used as necessary. In addition to these components, the aqueous liquid for the present invention may incorporate any additive for aqueous mixtures for padding of ordinary composition. Such additional additives include ultraviolet absorbents, antioxidants, antistatic agents, flame retardants, antiseptics, repellents, insecticides, resin cross-linking agents, surfactants, viscosity regulators, wetting agents, plasticizers, softening agents, perfumery, antibacterial deodorants, ordinary dyes and pigments, ultraviolet developing dyes, fluorescent pigments, phosphorescent pigments, luminous pigments, fluorescent brightening agents, extender pigments, electrolytes, resisting agents and discharging agents (anti-dyeing agents), thermosetting resins, and dryness regulators. These substances may be present in the above-described microcapsules, as long as they do not disturb the color changing properties of the microcapsules.

According to the coloring method of the present invention, a thermochromic and/or photochromic textile product, i.e., a colored product of the present invention, can be obtained by serially dipping a lengthy continuous textile product via a guider or the like in a padding bath in a padding machine containing the above-described aqueous liquid, to impart a color, dewatering (nipping) the thus-treated textile product using a mangle or the like, and then drying it using a tentering machine or the like. This mode of embodiment is nothing more than an example embodiment of the coloring method of the present invention. Other embodiments are possible, including enrichment of color variation by pre-drying the textile product after the first padding, then treating it by second padding wherein the textile product is dipped in a second padding bath containing microcapsules of a kind other than that of the microcapsules contained in the padding bath of the first padding, nipped, and then dried. One of the other embodiments is enhancement of the rubbing fastness of the colored product by treating the textile product by second padding wherein the product is dipped in a second padding bath containing the above-described thermoplastic resin as the only major component.

Examples of fibers constituting the lengthy continuous textile product for the present invention include cellulose fibers, such as cotton and hemp, protein fibers, such as wool and silk, regenerated fibers, such as viscose rayon and cupra, semi-synthetic fibers, such as acetate and triacetate, and synthetic fibers, such as polyamide, polyester, polyurethane, polyolefin, and acrylic. These fibers may be used in combination.

Examples of pieces of textile products comprising these fibers include sheet-form products and bundle-form products as described below.

The term "sheet-form product" mentioned herein is used in contrast to the term "bundle-form product" descried below. Specifically, it means a lengthy piece of cloth, such as a woven fabric, knitted fabric, or non-woven fabric, which can be used in a single continuous process. It is preferable that these forms of cloth be used in widths of scores of centimeters to several meters and in lengths of over scores of meters, from the viewpoint of productivity. However, shorter pieces of cloth may be simply sewed tentatively to yield a lengthy cloth for use in the present invention.

The term "bundle-form product" is used in contrast to the term "sheet-form product" described above, and is not subject to limitation, as long as it can be used in a serial coloring process, as described above. Such bundles include linearly formed products, such as yarns, strings and ropes, and several to several hundreds of such linearly formed products may be bundled or twisted together. Although it is preferable that these bundles be used in lengths of over scores of meters, shorter linearly formed products may be gently tied to an appropriate length. In addition, these textile products may be used after being colored previously.

The preferable subject of the present invention is a lengthy continuous textile product which is longitudinally uniform. The particularly preferable textile product for the present invention is a knitted fabric.

### EXAMPLE

The present invention is hereinafter described in more detail by means of the following examples, which are not to be construed as limitative.

In the following description, "part(s) by weight" are simply referred to as "part(s)".

### Preparation of thermochromic microcapsules

Crystal violet lactone (acid developing substance) 1 part
Bisphenol A (acidic substance) 3 parts
Myristyl alcohol (solvent) 25 parts

The above components were mixed together and thermally molten. This mixture was added to 200 parts of an 80°C aqueous solution containing 5 parts of CMC [carboxymethylcellulose] and 0.1 part of an anionic surfactant (product of Kao Corporation, trade name: Demol N), while stirring the solution, and emulsified until a mean particle size of about 3 µ m was obtained as confirmed by visual inspection (microscopy) (basic emulsification).

To this emulsion was added 15 parts of a 20% aqueous solution of a melamine-formalin prepolymer obtained by initial polymerization of 30 parts of granular melamine resin and 10 parts of formalin. After this mixture was adjusted to pH 5 with a 10% aqueous acetic acid solution, 5 parts of formalin was added, and the liquid temperature was raised to 95°C , followed by stirring for 2 hours to complete the reaction.

The thus-obtained dispersion liquid of thermochromic microcapsules was applied to a laser diffraction/scattering particle size distribution analyzer (product of Horiba, Ltd., model number: LA-700); the volume-based median diameter was determined to be 2.25 µ m. This dispersion liquid was filtered, and the filter cake was dried, to yield 30 parts of thermochromic microcapsules having a volume-based median diameter of 2.25µ m (thermochromic microcapsules A).

Also, thermochromic microcapsules B through K were prepared in the same manner as above, except that the particle size in the basic emulsification was adjusted to about 0.1 µ m, 0.3µ m, 0.5µ m, 1µ m, 5µ m, 8µ m, 12 µ m, 15 µ m, 17 µ m and 25µ m, respectively. Table 1 gives measurements of the volume-based median diameters of these microcapsules.

**TABLE 1**

| Thermochromic microcapsule | Volume-based median diameter |
|---|---|
| B | 0. 12 µm |
| C | 0. 28 µm |
| D | 0. 65 µm |
| E | 1. 27 µm |
| F | 4. 12 µm |
| G | 7. 93 µm |
| H | 10. 07 µm |
| I | 14. 85 µm |
| J | 16. 35 µm |
| K | 27. 83 µm |

### Preparation of photochromic microcapsules

3,3-diphenyl-3H-naphtho[2,1-b]pyran (organic photochromic compound) 1 part
1:1:1 methyl methacrylate : butyl methacrylate : acrylonitrile copolymer resin (molecular weight about 150,000) 10 parts
Diisononyl phthalate 20 parts
Xylene 15 parts
Epoxy resin (product of Yuka Shell Epoxy Co., trade name: Epikote 828) 4 parts
The above components were mixed together and thermally molten. This mixture was added to 700 parts of a 60 °C 10% aqueous gelatin solution, while stirring the solution, and emulsified until a mean particle size of about 3µ m was obtained as confirmed by visual inspection (microscopy) (basic emulsification). To this emulsion, 2 parts of an epoxy resin hardener (product of Yuka Shell Epoxy Co., trade name: Epomate B-002) was added. The liquid temperature was then raised to 80 °C, followed by stirring for 1 hour to complete the reaction.

The thus-obtained dispersion of photochromic microcapsules was applied to a laser diffraction/scattering particle size distribution analyzer (product of Horiba, Ltd., model number LA-700); the volume-based median diameter was determined to be 2.08 µ m. This dispersion was filtered, and the filter cake was dried, to yield about 50 parts of photochromic microcapsules having a volume-based median diameter of 2.08µ m (photochromic microcapsules A).

Also, photochromic microcapsules B through K were prepared in the same manner as above, except that the particle size at the basic emulsification was adjusted to about 0.1 µ m, 0.3µ m, 0.5µ m, 1µ m, 5µ m, 8µ m, 12 µ m, 15 µ m, 17 µ m and 25µ m, respectively. Table 2 gives measurements of the volume-based median diameters of these microcapsules.

**TABLE 2**

| Photochromic microcapsule | Volume-based median diameter |
|---|---|
| B | 0. 11 µm |
| C | 0. 35 µm |
| D | 0. 53 µm |
| E | 0. 98 µm |
| F | 3. 85 µm |
| G | 6. 98 µm |
| H | 11. 55 µm |
| I | 14. 94 µm |
| J | 15. 88 µm |
| K | 30. 03 µm |

### Example 1

50 kg of a cotton knitted fabric (grey sheeting, 50 cm width × 300 m length), circularly knitted with a previously scoured 20w cotton yarn, was unrolled, and passed through a padding bath [100 parts of water, 10 parts of thermochromic microcapsules A and 20 parts of an acrylic acid ester copolymer (thermoplastic resin) emulsion (50% aqueous emulsion of 2:1:1 ethyl acrylate : butyl acrylate : 2-ethylhexyl acrylate copolymer)] in a roll padder, and subsequently dewatered (nipped) to a squeezing rate of 100% using a mangle, followed by contactless drying at a temperature between 100 and 120 °C using a tentering machine, to thermochromically color the knitted fabric. The cotton knitted fabric thus colored with thermochromic microcapsules A developed a dense blue color at temperatures below 22 °C and a white color essential in cotton knitted fabrics at temperatures above 32 °C ; this color change phenomenon was reversibly repeatable. Also, this cotton knitted fabric showed substantially no hue difference or density difference transversely or longitudinally, demonstrating high uniformity, and its handling touch, appearance, rubbing fastness and washing fastness were excellent.

### Examples 2 through 7

The same procedure as in Example 1 was followed, except that thermochromic microcapsules A was replaced with thermochromic microcapsules D, E, F, G, H and I, respectively, to yield thermochromic cotton knitted fabrics.

The cotton knitted fabrics thus obtained, like the cotton knitted fabric of Example 1, developed a dense blue color at temperatures below 22°C and a white color essential in cotton knitted fabrics at temperatures above 32°C ; this color change phenomenon was reversibly repeatable. Data on various properties of these cotton knitted fabrics, along with those of the cotton knitted fabrics of Example 1, are shown in Table 3 below.

### Comparative Examples 1 through 4

The same procedure as in Example 1 was followed, except that thermochromic microcapsules A was replaced with thermochromic microcapsules B, C, J and K, respectively, to yield thermochromic cotton knitted fabrics. Data on various properties of these cotton knittings are shown in Table 3 below.

From Table 3, it is evident that these cotton knitted fabrics were inferior to the thermochromic cotton knitted fabrics of Examples 1 through 7 in commercial value, with lower color densities at temperatures below 22°C , ununiform coloring, and lower rubbing fastness and washing fastness.

The maximum color density values given in Table 3 were obtained at 20°C using a color difference meter model CR121 made by Minolta Camera Co, Ltd., and shown in percent ratios to the measurement in Example 1.

Figures for color difference were obtained at 20°C using the above-mentioned color difference meter.

Rubbing fastness was tested using a grey scale in accordance with AATCC8-1979; washing fastness was tested using a gray scale in accordance with the JIS L-0844 A-2 method.

**TABLE 3**

| | Used thermochromic microcapsule | Volume-based median diameter | Maximum color density value | Uniformity in the latitudinal direction [maximum color difference (ΔE)] | Uniformity in the longitudinal direction [maximum color difference (ΔE')] | Rubbing fastness | Washing fastness |
|---|---|---|---|---|---|---|---|
| Example 1 | A | 2.25 µm | 100% | ΔE<1 | ΔE' <1 | grade 3 | grade 3 |
| Example 2 | D | 0.65 µm | 95% | ΔE<1 | ΔE' <1 | grade 3 | grade 3 |
| Example 3 | E | 1.27 µm | 98% | ΔE<1 | ΔE' <1 | grade 3 | grade 3 |
| Example 4 | F | 4.12 µm | 103% | ΔE<1 | ΔE' <1 | grade 3 | grade 3 |
| Example 5 | G | 7.93 µm | 102% | ΔE<1 | ΔE' <1 | grade 3 | grade 3 |
| Example 6 | H | 10.07 µm | 100% | ΔE<1 | ΔE' <1 | grade 3 | grade 3 |
| Example 7 | I | 14.85 µm | 98% | ΔE<1 | ΔE' <1 | grade 3 | grade 3 |
| Comparative Example 1 | B | 0.12 µm | 25% | ΔE<1 | ΔE' <1 | grade 3 | grade 3 |
| Comparative Example 2 | C | 0.28 µm | 65% | ΔE<1 | ΔE' <1 | grade 3 | grade 3 |
| Comparative Example 3 | J | 16.35 µm | 71% | ΔE>2 | ΔE' >3 | grade 2 | grade 2 |
| Comparative Example 4 | K | 27.83 µm | 55% | ΔE>5 | ΔE' >7 | grade 1 | grade 1 |

### Example 8

300 m (100 kg) of a woven fabric of 90 cm in width, knitted with previously scoured pure silk, was dipped in a padding bath consisting of 100 parts of water, 8 parts of photochromic microcapsules A, 15 parts of a polyurethane resin (thermoplastic resin) emulsion (product of Dainippon Ink & Chemicals, Inc., trade name: HYDRAN HW311) and 3 parts of urea, using a roll padder, and subsequently dewatered (nipped) to a squeezing rate of 100% using a mangle, followed by contactless drying at a temperature between 100 and 120 °C using a tentering machine.

The thus-obtained photochromic silk woven fabric developed a white color essential in silk in a room not exposed to sunlight, and a dense yellow color by windows or outdoors with exposure to sunlight or under lighting with a UV fluorescent lamp; this color change phenomenon was reversibly repeatable. Also, this silk woven fabric showed substantially no hue difference or density difference transversely or longitudinally, demonstrating a uniform color development, and its handling touch, appearance, rubbing fastness and washing fastness were excellent.

### Examples 9 through 14

The same procedure as in Example 8 was followed, except that photochromic microcapsules A was replaced with photochromic microcapsules D, E, F, G, H and I, respectively, to yield photochromic silk woven fabrics.

The thus-obtained silk woven fabrics showed the same photochromic phenomenon as in Example 8, with excellent handling touch, appearance, rubbing fastness and washing fastness. Data on various properties of these silk woven fabrics, along with those of the silk woven fabric of Example 8, are shown in Table 4 below.

### Comparative Examples 5 through 8

The same procedure as in Example 8 was followed, except that photochromic microcapsules A was replaced with photochromic microcapsules B, C, J and K, respectively, to yield photochromic silk woven fabrics. Data on various properties of these silk woven fabrics are shown in Table 4 below.

From Table 4, it is evident that these silk woven fabrics were inferior to the photochromic silk woven fabrics of Examples 8 through 14 in commercial value, with lower color densities at the time of photochromic color development, ununiform coloring, and lower rubbing fastness and washing fastness.

The maximum color density values given in Table 4 were obtained at the time of light irradiation using a color difference meter model CR121 made by Minolta Camera Co, Ltd., and shown in percent ratios to the measurement in Example 8. Figures for color difference were obtained at the time of light irradiation using the above-mentioned color difference meter. Rubbing fastness and washing fastness were tested in the same manner as in Table 3.

**TABLE 4**

| | Used photochromic microcapsule | Volume-based median diameter | Maximum color density value | Uniformity in the latitudinal direction [maximum color difference (ΔE)] | Uniformity in the longitudinal direction [maximum color difference (ΔE')] | Rubbing fastness | Washing fastness |
|---|---|---|---|---|---|---|---|
| Example 8 | A | 2.08 µm | 100% | ΔE<1 | ΔE' <1 | grade 3 | grade 3 |
| Example 9 | D | 0.53 µm | 97% | ΔE<1 | ΔE' <1 | grade 3 | grade 3 |
| Example 10 | E | 0.98 µm | 99% | ΔE<1 | ΔE' <1 | grade 3 | grade 3 |
| Example 11 | F | 3.85 µm | 102% | ΔE<1 | ΔE' <1 | grade 3 | grade 3 |
| Example 12 | G | 6.98 µm | 102% | ΔE<1 | ΔE' <1 | grade 3 | grade 3 |
| Example 13 | H | 11.55 µm | 100% | ΔE<1 | ΔE' <1 | grade 3 | grade 3 |
| Example 14 | I | 14.94 µm | 98% | ΔE<1 | ΔE' <1 | grade 3 | grade 3 |
| Comparative Example 5 | B | 0.11 µm | 22% | ΔE<1 | ΔE' <1 | grade 3 | grade 3 |
| Comparative Example 6 | C | 0.35 µm | 69% | ΔE<1 | ΔE' <1 | grade 3 | grade 3 |
| Comparative Example 7 | J | 15.88 µm | 70% | ΔE>2 | ΔE' >3 | grade 2 | grade 2 |
| Comparative Example 8 | K | 30.03 µm | 44% | ΔE>5 | ΔE' >7 | grade 1 | grade 1 |

### Example 15

50 kg of a pink ground dyed circularly knitted blended fabric (grey sheeting, 200 m) of 35% polyester and 65% cotton, 90 cm in width, was dipped in a padding bath [100 parts of water, 8 parts of thermochromic microcapsules F, 8 parts of photochromic microcapsules F, 10 parts of an acrylic acid ester copolymer resin (thermoplastic resin) emulsion (product of Kanebo N.S.C Ltd., trade name: Yodosol MR-96) and 3 parts of a higher fatty acid ester-based softening agent (product of Meisei Chemical Works, Ltd., trade name: Eleganol HAS)] using a roll padder, and subsequently dewatered (nipped) to a squeezing rate of 100% using a mangle, followed by contactless drying at a temperature between 100 and 120 °C using a tentering machine.

This knitted fabric was further dipped in a padding bath [100 parts of water, 10 parts of an acrylic acid ester copolymer resin (thermoplastic resin) emulsion [product of Dainippon Ink and Chemicals, Inc., trade name: Voncoat R-3360)], and dewatered (nipped) to a squeezing rate of 100% using a mangle, followed by contactless drying at a temperature between 100 and 120 °C using a tentering machine.

The thus-obtained knitted fabric showed multiple color changes including pink, purple, orange and brown, depending on the presence or absence of light irradiation and temperature changes; this color change phenomenon was reversibly repeatable. Also, shirts obtained by cutting and sewing this knitted fabric showed the same multiple color change phenomenon as above, with good handling touch and appearance and further excellent rubbing fastness and washing fastness, demonstrating outstanding commercial value.

### Example 16

1 kg of a folded rayon yarn, consisting of ten pure rayon yarns of 2 denier, was dipped in a padding bath [100 parts of water, 0.2 parts of phthalocyanine blue (organic pigment), 12 parts of photochromic microcapsules F, 5 parts of glycerol, 15 parts of an acrylic acid ester copolymer (thermoplastic resin) emulsion (product of Matsui Shikiso Chemical Co., Ltd., trade name: Matsuminsol MR conc) and 0.5 parts of an ethylene urea condensation product (product of Matsui Shikiso Chemical Co., Ltd., trade name: Fixer F)] using a padding machine, and subsequently dewatered (nipped) to a squeezing rate of 100% using a mangle, followed by contactless drying at a temperature between 100 and 120 °C using a hot air drier.

This folded rayon yarn was further dipped in a padding bath [100 parts of water and 2 parts of a silicone-based softening agent (product of Matsui Shikiso Chemical Co., Ltd., trade name: Softener AQ)] using a padding machine, and subsequently dewatered (nipped) to a squeezing rate of 80% using a mangle, followed by drying at a temperature between 100 and 120 °C using a hot air drier, after which the yarn was wound up.

The color of thus-obtained photochromic rayon yarn was blue in a room not exposed to sunlight. But the rayon yarn developed a green color by windows or outdoors with exposure of sunlight; this color change phenomenon was reversibly repeatable. Moreover, this rayon thread showed a longitudinally uniform color density, with excellent rubbing fastness and washing fastness and good appearance and handling touch.

## Claims

1. Coloring method wherein a lengthy continuous textile product is serially treated with an agueous liquid containing a thermoplastic resin and thermochromic and/or photochromic microcapsules having a volume-based median diameter of 0.5µ m to 15 µ m by padding.

2. Coloring method of claim 1 wherein said textile product is further serially treated with another aqueous liquid containing a thermoplastic resin and other kinds of thermochromic and/or photochromic microcapsules having a volume-based median diameter of 0.5µ m to 15 µ m by padding

3. Coloring method of claim 1 wherein said textile product is further serially treated with another aqueous liquid containing a thermoplastic resin as the only major component by padding.

4. Coloring method of claim 2 wherein said textile product is further serially treated with another aqueous liquid containing a thermoplastic resin as the only major component by padding.

5. Colored product made by the coloring method of claim 1.

6. Colored product made by the coloring method of claim 2.

7. Colored product made by the coloring method of claim 3.

8. Colored product made by the coloring method of claim 4.
